

# UNITED STATES PATENT OFFICE.

OTTO RÖHM, OF DARMSTADT, GERMANY.

## PROCESS FOR SOFTENING HIDES, SKINS, OR THE LIKE.

1,257,402.

Specification of Letters Patent. Patented Feb. 26, 1913.

No Drawing.

Application filed August 27, 1915. Serial No. 47,626.

To all whom it may concern:

Be it known that I, OTTO RÖHM, a subject of the King of Wurttemberg, residing at Darmstadt, in the Grand Duchy of Hesse, have invented a new and useful Process for Softening Hides, Skins, or the like, of which the following is a specification.

In making furs it is necessary to well soften the raw hides and skins, which have mostly been previously air-dried. This is done, partly by allowing the hides to putrify for a few days, and partly by soaking them in a solution of soda and soap in water. By this means the superficially adhering dirt is removed, the flesh and fat adhering to the flesh side is loosened, which must be removed before the tanning process is carried out, and the fiber of the hide is well softened, so that it can take up the tanning material and produce a soft leather.

I have found that this softening and cleaning of the hides and skins will be carried out much better and more quickly than with the old process if the hides are placed in a solution of the enzymes (ferments) of the pancreatic gland of animals. The softening process is then mostly concluded in one day, even in the case of hard dried hides, which often require 4-8 days soaking. A further advantage consists in the fact that the fat is easily loosened and the absorption of the tanning material is accordingly facilitated. Moreover the flesh becomes quite tender, and it can then be easily scraped off with a knife. An economy of time is thus effected and there is no danger of holes being cut in the hides as when they have to be strongly treated with the knife in order to remove the flesh. Care must be taken to interrupt the process in good time, because, if carried out too long and too strongly, the hairs are loosened. I have also found that the injury done to the hairs and wool is

greater according as the reaction of the enzyn solution is more neutral. All injury to the hairs and wool is completely avoided if the solution is sufficiently alkaline. For example, good results are obtained with a solution of 0.05% pancreatin and 1% soda ash in water. The proper alkaline character of the solution can be obtained in other ways, and enzymes, which dissolve fat and albumen, of other sources can be used. The process can, of course, also be employed with great advantage for softening hides and skins which are not to be made up into furs, but are to be used as common leather.

What I claim and desire to secure by Letters Patent of the United States is:—

1. The process for softening raw hides, skins and the like which process consists in treating the same in a solution of water and enzymes of the pancreatic gland of animals dissolving fat and albumen.

2. The process for softening raw hides, skins and the like which process consists in treating the same in a solution of water and enzymes of the pancreatic gland of animals dissolving fat and albumen and of so strongly alkaline character that no injury is done to the hairs and wool.

3. The process for softening hides, skins, and the like, which consists in treating the same in a solution of water and enzymes of the pancreatic gland of animals dissolving fat and albumen, said solution consisting of water containing 0.05% pancreatin and 1% of soda ash.

In testimony whereof, I have signed my name to this specification in the presence of two subscribing witnesses.

OTTO RÖHM.

Witnesses:

HUGO KARP,  
ERNST SCHÄUDLER.